

## UNITED STATES PATENT OFFICE

2,317,965

## PROCESS OF COLORING FIBROUS MATERIALS AND THE MATERIALS OBTAINED THEREBY

Herbert Bestian, Joseph Nüsslein, and Josef Monheim, Frankfort-on-the-Main, Germany, assignors to General Aniline & Film Corporation, New York, N. Y., a corporation of Delaware

No Drawing. Application April 27, 1940, Serial No. 332,015. In Germany May 27, 1939

2 Claims. (Cl. 8—74)

The present invention relates to a process of coloring fibrous materials and to the materials obtained thereby.

We have found that colored effects may be produced on materials of fibrous structure by treating the fibrous materials at any stage of the coloring operation, i. e., before, during or after the coloring step with products of the general formula:



or the homologues or the derivatives thereof, wherein R stands for a member of the group consisting of aliphatic and isocyclic radicals, and then polymerizing the monomeric compound.

In their monomeric form, the said products are partly water-soluble and may be applied to the fibrous material in an aqueous solution. If the compounds are insoluble or difficultly soluble in water they may be used in the form of their aqueous suspensions or their solutions in organic solvents; also products which have already been partially polymerized may, if desired, be applied to the material. After the impregnation, the compounds are polymerized, suitably by a heat treatment, for instance at 100° C.—160° C. or a higher temperature, and in this way are incorporated with the fibrous material in a water-insoluble form. The polymerization may be carried through according to the processes described in U. S. Patents No. 2,265,416 issued December 9, 1941, and No. 2,312,863, issued March 2, 1943, both in the name of Herbert Bestian, for "Polymerization products."

As fibrous materials there are suitable fibers of vegetable or animal origin, furthermore fibers from regenerated cellulose or cellulose derivatives, also mineral or synthetic fibers, for instance glass or asbestos fibers, polyamide and polyvinyl chloride fibers and likewise leathers and hides.

By the new process there may be obtained, independently of the tinctorial behavior of the printed or padded materials, novel color effects as a result of the absorption capacity of the products applied for the coloring material. By taking advantage of the behavior of the said products and of the fibrous materials against dyestuffs different effects are obtained which may even be far more varied by altering the amount of the product applied and the temperature and duration of the heat-treatment and, if desired, by adding suitable compounds, for instance formaldehyde or compounds yield-

ing formaldehyde. The effects thus produced possess an excellent fastness to water and to washing.

Instead of subjecting the impregnated fibrous material to the heat-treatment it may be dried at temperatures below 100° C. and hot dilute acids or aqueous solutions of polyvalent electrolytes in the absence or presence of acids may be caused to act upon it. As electrolytes, there

10 may be used, for instance, the salts of iron, aluminum, nickel, cobalt, chromium, magnesium or calcium.

Cotton or regenerated cellulose may thus be treated with the compounds according to the 15 above-named formula which are to be considered as urea derivatives, and the compounds may be polymerized on the fiber. In this manner a material is obtained which possesses an increased absorption capacity for acid wool dyestuffs. The cellulose fibers thus pre-treated also show an improved affinity for the ordinary cotton dyestuffs, the so-called substantive dyestuffs; and the fastness to water and to washing of the dyeings thus obtained is considerably improved. Wool may likewise be pre-treated in the aforesaid manner and then shows an increased absorption capacity for acid dyestuffs. When pre-treating in the same manner fibrous materials from cellulose esters or ethers a material is obtained possessing an increased affinity for the so-called acetate silk dyestuffs, besides an affinity for acid wool dyestuffs. Furthermore, the treatment with the above-named products may replace the previous mordant operation in the dyeing of cotton with basic dyestuffs or with mordant dyestuffs.

The above-named products may likewise be applied on textile materials simultaneously with dyeing bodies and then firmly be fixed on the 40 material by a thermal after-treatment. In this manner, there may be obtained vivid dyeings and prints, for instance by padding, spraying and printing fabrics from cotton or regenerated cellulose with solutions or suspensions of acid wool dyestuffs and of urea derivatives which, when dyestuffs capable of being discharged are used, may be discharged in known manner so as to obtain white or colored effects.

Also colored or white pigments may be fixed on 50 the fibrous material by means of urea derivatives. For instance, aqueous solutions of the products named are mixed with pigments such as titanium dioxide, soot, ultramarine, iron oxide or organic pigments such as azo-dyestuffs insoluble in water, and applied on cotton or regenerated cellulose by padding, spraying or printing. After pol-

Ymerization of the urea compounds the pigments are firmly fixed on the material. The dyeings or prints so obtained are very stable against the usual washing processes. It is not always necessary to apply to the fibrous material a mixture of the pigment dyestuff and the urea derivative, but the pigment dyestuff may also be prepadded, dried and cross-padded with the solution of the urea derivative. This process of fixing pigments on fibrous materials is especially suitable for uniformly coloring mixed fabrics or mixed structures, for instance union or halfsilk or mixtures from regenerated cellulose and other fibrous materials which do not possess uniform affinity for dyestuffs.

Dyeings on cellulose with substantive dyestuffs, which dyeings in many cases show an insufficient fastness to water and to washing may be improved as to their fastness to water and to washing by impregnating them with the urea derivatives in question, for instance by cross-padding. Fastness properties are obtained thereby which are considerably more improved than in the case of after-treating the dyeings by means of highly molecular amines or ammonium compounds. Dyeings with other dyestuffs, for instance with mordant dyestuffs on cellulose may likewise be improved as to their fastness to water and to washing by after-treating them as described above.

The monomeric starting compounds may be obtained by reaction of aliphatic, cycloaliphatic, aromatic and araliphatic diisocyanates with ethylene imine or the homologues thereof. For instance, by the reaction of ethylenimine or the homologues and derivatives thereof with aliphatic, aromatic, araliphatic or cycloaliphatic di-isocyanates there may, under suitable working conditions, be obtained products of the general formula:



wherein R stands for a substituent of the group consisting of arylene, alkylene, aralkylene, cycloalkylene and alkylenes the chains of which contain hetero atoms, and  $X_1$ ,  $X_2$ ,  $X_3$ ,  $X_4$  stand for substituents of the group consisting of hydrogen, alkyl, aryl and aralkyl.

As starting substances there may, for instance, be used compounds the radical  $-R-$  of which has the following constitution:



the radical may likewise be branched, for instance



as well as the corresponding metal-and para-compounds.



5

10 as well as the corresponding meta- and para- compounds and bromine compounds.



20. as well as the corresponding bromine compound:



40 The radical —R— may likewise be interrupted by hetero atoms, for instance:



or



The hydrogen atoms of the ethylene groups may partly or entirely be substituted by methyl, ethyl, propyl, isopropyl, butyl, isobutyl, amyl, iso-  
50 amyl, decyl, furthermore by phenyl, the methyl-phenyl radicals, benzyl and —ortho—, —meta— and —para—tolyl. Two, three or all of the four hydrogen atoms may likewise be substituted by two, three or four different substituents as named above.

The following examples serve to illustrate the invention, but they are not intended to limit it thereto:

60 1. A cotton fabric is printed with a thickened solution of 20 per cent. strength of the reaction product of hexamethylene-diisocyanate and ethyleneimine, dried for 8 minutes at 140° C. and dyed with the dyestuff No. 363 (Schultz, "Farbstoff tabellen," 7th edition). The printed parts are dyed vivid pink tints and the dyeing has a good fastness to washing. Similar results are obtained on fabrics from viscose-, cuprammonium- and acetate artificial silk, artificial silk staple fiber and linen. On using a cotton ground previously dyed with substantive dyestuffs there are obtained two-color- or intensive half-tone effects, according to the ground color used.

2. Glass wool is impregnated with the reaction product from octamethylene-diisocyanate and

ethyleneimine, dried and heated for 5 minutes to 180° C.-200° C. By means of the azo-dyestuff



3. When cotton is printed with the reaction product from octamethylene-diisocyanate and ethyleneimine, dried for 5 minutes at 130° C.-145° C. and dyed with sulfonated 4,4'-diaminodianthrimide without the addition of a chromium salt, a deep-black dyeing of the print is obtained which is fast to washing. A chromium salt may likewise be used, and in this case it is of little difference only, whether the chromium salt is applied before, during or after the dyeing operation.

4. A fabric from artificial silk staple fiber is padded with an aqueous solution of 15 per cent. strength of the reaction product from tetramethylene-diisocyanate and ethylene-imine and dried for a short time at 130° C.-145° C. The material is then dyed with the dyestuff obtained by condensation of para-chlorobenzaldehyde and ethyl-benzyl-meta-toluidine, trisulfonation, oxidation and melting with para-phenetidine and a vivid blue dyeing is obtained which is fast to water and to washing. The blue dyeing thus obtained may be discharged by means of formaldehyde-sulfoxylate to a white which does not change color. If instead of the blue dyestuff the dyestuff No. 732 (Schultz, I. c.) is used, a brilliant strong yellow dyeing is obtained. If the latter is printed with a discharge preparation containing the dyestuff No. 1330 (Schultz, I. c.), steamed for 5 minutes in a rapid ager, rinsed and soaped, a deep-blue discharge print is obtained on a yellow ground.

5. A viscose artificial silk fabric is padded with an aqueous solution of 20 per cent. strength of the reaction product named in Example 1, dried at 60° C. and overprinted with a printing paste containing an acid or an acid salt, for instance acetic acid or aluminium sulfate. Thereupon, the material is heated to 140° C., dyed with the azo-dyestuff acetyl-cyclohexyl-para-phenylenediamine  $\rightarrow$  benzoyl-K-acid and soaped for a short time. Half-tone resists are obtained on a red ground.

6. A fibrous material of polyvinyl chloride is padded with a solution of the reaction product from hexamethylene-diisocyanate and ethyleneimine and the chromium complex compounds of the azo-dyestuffs from diazotized 1-amino-2-hydroxy-3-nitrobenzene-5-sulfonic acid and beta-naphthylamine, dried for 20 minutes at 80° C., treated for 20 minutes at 70° C. in a bath containing per liter of water 50 cc. of concentrated sulfuric acid and 3 grams of cobalt nitrate, and rinsed. The material is dyed intense green shades.

7. Fabrics from mercerized or unmercerized cotton are printed as described in Example 1, heated for 8 minutes to 140° C. and dyed with the dyestuff obtained by condensation of dinitrostilbene-disulfonic acid with the azo-dyestuff para-sulfanilic acid  $\rightarrow$  alpha-naphthylamine. The printed parts show deeper shades than the ground and the dyeings obtained are distinctly faster to washing than the ground dyeings.

After having been printed according to Example 1 and heated for 8 minutes to 140° C. chlorinated or unchlorinated wool may likewise be dyed with the dyestuff No. 603 (Schultz, I. c.).

The printed wool may also be intensely dyed with the dyestuff obtained by condensation of dinitrostilbene-disulfonic acid with the azo-dyestuff para-sulfanilic acid  $\rightarrow$  alpha-naphthylamine.

5. Acetate silk, which has been pre-treated as described in Example 1 and subsequently heated, may likewise be dyed with the azo-dyestuff 2,6-dichloro-4-nitraniline  $\rightarrow$  N-hydroxyethyl-N-methyl-meta-toluidine.

10. By adding to the printing paste 10 per cent. of formaldehyde of 40 per cent. strength or paraformaldehyde the time of heating may be considerably shortened.

8. A cotton fabric printed according to Example 1 is heated for 5 minutes to 100° C. or steamed in a rapid ager, dyed with the disazo-dyestuff 4,4'-diaminodiphenyl-3,3'-bisglycolic acid  $\rightarrow$  para-anisidyl-J-acid and subsequently treated with a copper sulfate solution. A dark-blue print which is fast to washing is obtained on a blue ground.

9. Muslin from artificial silk staple fiber is printed as described in Example 3, dried at 100° C., dyed with the dyestuff obtained by reduction of the azo-dyestuff

25.  $\text{paranitraniline} \xrightarrow{\text{acid}}$  1,8-aminonaphthol-4,6-disulfonic acid  
and reaction with phosgene, and coupled with diazotized para-nitraniline. After soaping the material, a dark-green print is obtained on a green ground.

10. A material padded according to Example 4 is dried at 100° C. and dyed with the dyestuff



The dyeing obtained has a good fastness to 40. washing and is dischargeable to a white.

11. Muslin from artificial silk staple fiber padded as described in Example 5 is heated for 10 minutes to 140° C. and dyed with the azo-dyestuff 4-amino-azobenzene-4'-sulfonic acid  $\rightarrow$  para-aminobenzoyl-meta-aminobenzoyl-J-acid. The dyeing thus obtained is distinctly more yellowish than a corresponding dyeing produced on a not pre-treated material and possesses a far better fastness to water and to washing. In comparison 50. with a dyeing on a not pre-treated material which has been diazotized and developed with beta-naphthol the shade of the dyeing obtained as above is somewhat more bluish and shows an improved fastness to water.

55. 12. A print produced according to Example 3 is heated for some minutes, on the felt calender, to 135° C. and dyed with the dyestuff obtainable according to Example 2 of U. S. Patent No. 2,044,963 with use of para,para'-tetra-hydroxyethyldiamino-meta,meta'-dimethylbenzophenone, and with alum. The printed parts are dyed deep-blue tints. Instead of alum there are likewise suited other salts, for instance copper and cobalt salts.

60. 13. Prints, produced as described in Example 1 and heated to 140° C., are dyed with the dyestuff No. 1145 (Schultz, I. c.). Red-brown tints of good fastness to washing are obtained. If the prints are previously mordanted with formic acid or with formic acid and potassium di-chromate current shades are obtained on dyeing. On previously mordanting with alum, tartar and oxalic acid yellowish red tints are obtained.

65. 14. Prints on cotton produced according to Example 1 are steamed for 5 minutes in a rapid

ager, treated for a short time in a hot bath containing 2 per cent. of formic acid and 2 per cent. of cobalt nitrate and dyed with the azo-dyestuff 1-sulfanilido-2-para-toluidine-1,4-naphtholsulfonic acid, an intense red dyeing of the printed parts being obtained thereby. On addition of hexamethylenetetramine to the printing paste deeper shades may be obtained.

15. A mixed fabric consisting of viscose and cotton, which fabric tends to become streaky on dyeing, is padded with an aqueous solution containing 10 per cent. of the reaction product described in Examples 1 and 3 per cent. of the dyestuff No. 189 (Schultz, I. c.) and heated for 5 minutes to 140° C. A vivid, uniform orange dyeing is obtained which may be discharged to a white. The padding solution may likewise be used with advantage in spray printing.

16. A printing color consisting of 10 grams of the reaction product according to Example 1, 2 grams of the dyestuff mentioned in Example 5 of German Patent No. 293,352, 53 grams of neutrugacanth thickening and 35 grams of water is printed on dulled cuprammonium silk or on a fabric of asbestos fiber, steamed in a rapid ager for 10 minutes and rinsed. The prints obtained have vivid shades and a good fastness to washing.

17. Cotton material dyed with the dyestuff No. 306 (Schultz, I. c.) is padded with an aqueous solution of 10 per cent. strength of the reaction product mentioned in Example 1, dried and heated for a few minutes to 140° C. This treatment renders the color shades more yellow and distinctly clearer. The fastness to wet processing, particularly to washing at 100° C., is essentially improved thereby. By treating material dyed with the dyestuff No. 510 (Schultz, I. c.) in the same manner there is likewise obtained a dyeing having a considerably better fastness to washing.

18. If a dyeing on tannin-mordanted artificial silk staple fiber, dyed with the dyestuff used in Example 12, is after-treated as described in Example 17 the fastness to washing of the dyeing obtained is quite essentially improved.

19. A cotton fabric is padded with a liquor containing 5 per cent. of the dyestuff No. 86 (Schultz, I. c.), 10 per cent. of the reaction product mentioned in Example 1, 1 per cent. of high-

ly polymerized polyvinyl alcohol and 84 per cent. of water, dried and heated for 5 minutes to 140° C. A brilliant red dyeing of very good fastness to washing is obtained. The fabric may also be padded with the pigment dyestuff and after drying may further be padded with the solution of the above-named reaction product. It is then dried and subsequently heated as described above. Thereby a dyeing is obtained which is particularly fast to rubbing.

We claim:

1. The process of coloring fibrous materials which comprises applying to the material at any stage of the coloring operation a compound of the general formula



wherein R stands for a member of the group consisting of alkylene, arylene, aralkylene, cycloalkylene and alkylenes the chains of which contain hetero atoms, and X<sub>1</sub>, X<sub>2</sub>, X<sub>3</sub> and X<sub>4</sub> stand for substituents selected from the group consisting of hydrogen, alkyl, aryl and aralkyl radicals and polymerizing the monomeric compound.

2. Fibrous materials carrying a polymer of a compound of the general formula



wherein R stands for a member of the group consisting of alkylene, arylene, aralkylene, cycloalkylene and alkylenes the chains of which contain hetero atoms, and X<sub>1</sub>, X<sub>2</sub>, X<sub>3</sub> and X<sub>4</sub> stand for substituents selected from the group consisting of hydrogen, alkyl, aryl and aralkyl radicals and a coloring agent.

HERBERT BESTIAN.  
JOSEPH NÜSSLEIN.  
JOSEF MONHEIM.